

1

2,784,084

## ZIRCONIUM TERNARY ALLOYS

Lyle L. Marsh, Jr., and Walston Chubb, Columbus, Ohio, assignors to the United States of America as represented by the United States Atomic Energy Commission

No Drawing. Application July 12, 1954,  
Serial No. 443,984

1 Claim. (Cl. 75—177)

The present invention is concerned with zirconium base alloys and particularly with zirconium-niobium base ternary alloys.

The development of nuclear reactors for power applications and of cyclotrons, linear accelerators and similar apparatus subject to radioactivity and high temperatures has caused a demand for novel alloys having good high-temperature strength and low neutron absorption characteristics for structural members in such apparatus. The strength characteristics of these new alloys should be approximately as good as the characteristics of the stainless steels normally used in high-temperature devices but the alloys should have a much lower neutron capture cross section than the stainless steels. Furthermore, the alloys must have sufficient workability to enable them to be fabricated into simple shapes.

While such elements as aluminum, lead, molybdenum, niobium, tantalum, tin, titanium and vanadium can all be used to strengthen zirconium effectively in binary alloys, it has been found in general that reasonable strength can be achieved only by sacrificing ductility or by increasing the thermal-neutron capture cross section of the alloy to an undesirable extent. This results from the fact that no element has been found as yet which has the combination of a high solubility in alpha zirconium, a low thermal-neutron capture cross section, and a satisfactorily high boiling point.

It is an object of the present invention to provide novel alloys having tensile characteristics at high temperatures approximately equivalent to that of stainless steel and satisfactory ductility characteristics at high temperatures, but having capture cross sections for thermal-neutrons less than one-third the capture cross section of stainless steel.

In accordance with the present invention it has been found that novel zirconium base ternary alloys containing niobium and a third metal from the group consisting of aluminum, molybdenum, and vanadium have very desirable tensile characteristics at high temperatures; have low thermal-neutron capture cross sections and have highly desirable ductility characteristics. The niobium component of these ternary alloys can be present in from about 1 to 5 w/o (weight percent) and the third metallic component may be present in 0.1 to 2 w/o. The term "zirconium-niobium ternary alloy" refers herein to an alloy comprised primarily of three metallic components

2

wherein zirconium is the predominant component and the weight percent of niobium present exceeds the weight percent of the third metallic component.

Zirconium is a transition element characterized by an incomplete inner shell of *d* electrons and an allotropic transformation at 865° C., transforming from a hexagonal crystal structure into a high-temperature body-centered cubic structure. The three minor components of the ternary alloys, namely, aluminum, vanadium, and molybdenum all have interatomic distances less than that of zirconium and lying within the range of the Hume-Rothery Rule. The percent difference of the interatomic distance of the third component from that of zirconium is: aluminum, -10%; molybdenum, -13%; and vanadium, -16%. It may be noted that the percent difference of the interatomic distance of niobium compared to that of zirconium is -9%.

The alloys may be produced by conventional methods. For the experiments described below the alloys were prepared by drilling holes in pieces of metallic zirconium, putting suitable quantities of the two minor components into these holes and then filling the holes with zirconium chips. These zirconium pieces were then heated in a graphite crucible by high-frequency induction at an absolute pressure of less than 10 microns of mercury. A charge of about 200 grams is melted in each case; the crucible is first charged with about half this quantity and after this first portion has melted the remainder of the charge is added. The melted alloys are then allowed to cool slowly. The ingots obtained thereby weigh between 160 and 180 grams, part of the material having been taken up by the graphite of the crucible.

The alloys were also produced in arc-melting furnaces and satisfactory results were obtained by this method. During the melting in the graphite crucibles a small amount of carbon, up to about 0.5% by weight, was picked up by the alloys. A comparison of the high-temperature tensile strength of the alloys showed a very definite trend in favor of the arc-melted alloys over the induction-melted alloys. This may be caused in part by the strengthening effect of the small amount of carbon present.

The various alloys produced were tested at 500° C. for hardness, tensile strength, and elongation, the characteristics primarily of interest for structural materials. For the hardness tests the ingots of the alloys were first upset-forged and then hot-rolled at 1000° C. to yield  $\frac{1}{8}$ -inch thick slabs. Then about 0.01 inch of the slabs was shaved off from the surface on each side in order to remove any gaseous contaminants. The "scalped" slabs were then cold-rolled in reductions of approximately 0.002 inch per pass until a total reduction of from 20 to 30% had been obtained. The cold-rolled alloys were then annealed for one hour at 700° C. in a straightening press. The sheets resulting thereby were again "scalped" 0.018 inch on one side and cut into testing specimens. The hardness was determined at three stages of the alloys, namely, as-cast, cold-rolled, and annealed, and the results are tabulated in the following table.

TABLE I  
Hardness data for zirconium alloys

| Alloy Analysis, w/o | Hardness, Rockwell A |                       |                  |                    |
|---------------------|----------------------|-----------------------|------------------|--------------------|
|                     | As Cast              | As Rolled at 1,000°C. | Cold Rolled, 40% | Annealed at 700°C. |
| 1.0 Nb+0.5 Al       | 58                   | 61                    | 60               | 55                 |
| 1.5 Nb+1.0 Al       | 56                   | 62                    | 61               | 56                 |
| 1.8 Nb+0.6 Mo       | 53                   | 58                    | 60               | 53                 |
| 1.4 Nb+1.1 Mo       | 55                   | 68                    | 60               | 54                 |
| 2.0 Nb+1.6 Mo       | 68                   | 69                    | 63               | 60                 |
| 1.0 Nb+0.3 V        | 49                   | 58                    | 60               | 52                 |
| 1.3 Nb+1.1 V        | 52                   | 61                    | 62               | 53                 |
| 2.2 Nb              | 59                   | 61                    | 57               |                    |
| 6.0 Nb              | 63                   | 66                    | 58               | 58                 |

<sup>1</sup> Rolled less than 10%.

For the tensile strength tests, specimens 5 inches long,  $\frac{5}{16}$  inch wide, and 0.04 to 0.08 inch thick were prepared. The reduced section was 1.5 inches long and  $\frac{1}{16}$  inch wide. The specimens were tested at 500° C. in an argon atmosphere. The speed of travel of the head of the testing machine was 0.02 inch per minute and an extensometer with a one-inch gauge length and an accuracy of plus or minus 0.0001 inch per inch was used to measure extensions. The extensometer was of the clip-on type with slide bars extending out of the heated area around the specimen.

The results of these tensile tests are shown in Table II. The tests were run in duplicate on each alloy and the results shown in Table II represent the average values obtained from these tests. The values listed under "uniform elongation" represent the total elastic and plastic deformation at maximum load. The tensile strength of the zirconium-niobium binary alloy is shown for purposes of comparison.

and thermal-neutron capture cross section of these materials with those of stainless steel, zirconium and zirconium-niobium binary alloys. These are shown in Table III.

TABLE III  
Properties of zirconium alloys compared with properties of stainless steel at 500° C.

| Alloy Analysis, w/o<br>(Balance Zr)                    | Thermal-<br>Neutron<br>Capture<br>Cross<br>Section, <sup>1</sup><br>barns/atom | Cross<br>Section<br>Ratio <sup>2</sup> | Yield<br>Strength<br>Ratio <sup>3</sup> |
|--------------------------------------------------------|--------------------------------------------------------------------------------|----------------------------------------|-----------------------------------------|
| Type 347 Stainless Steel<br>Induction-Melted Zirconium | 2.86                                                                           | 1                                      | 1                                       |
| 1.0 Nb+0.5 Al                                          | 0.18                                                                           | 0.063                                  | 0.3                                     |
| 1.5 Nb+1.0 Al                                          | 0.19                                                                           | 0.066                                  | 0.85                                    |
| 1.8 Nb+0.6 Mo                                          | 0.19                                                                           | 0.066                                  | 1.11                                    |
| 1.4 Nb+1.1 Mo                                          | 0.20                                                                           | 0.070                                  | 0.57                                    |
| 2.0 Nb+1.6 Mo                                          | 0.21                                                                           | 0.074                                  | 0.68                                    |
| 2.0 Nb+1.6 Mo                                          | 0.24                                                                           | 0.084                                  | 0.95                                    |
| 2.0 Nb+1.6 Mo                                          | 0.21                                                                           | 0.074                                  | 0.53                                    |
| 1.3 Nb+1.1 V                                           | 0.27                                                                           | 0.094                                  | 0.66                                    |
| 2.2 Nb                                                 | 0.22                                                                           | 0.077                                  | 1.13                                    |
| 6.0 Nb                                                 | 0.23                                                                           | 0.080                                  | 1.17                                    |

<sup>1</sup> Based on 0.18 barn/atom for zirconium.<sup>2</sup> Based on 2.86 barns/atom for stainless steel.<sup>3</sup> Based on a yield strength of 31,000 p. s. i. for stainless steel at 500° C.

The 1.5 niobium plus 1.0 aluminum ternary alloy is particularly outstanding, both in regard to yield strength ratio which is better than type 347 stainless steel at 500° C., cross section ratio which is less than  $\frac{1}{10}$  as great as stainless steel, and ductility (as shown in Table II) which is several times better.

It will be understood that this invention is not to be limited to the details given herein but that it may be modified within the scope of the appended claim.

30 What is claimed is:

A ductile zirconium base alloy consisting essentially of

TABLE II

Tensile properties of zirconium alloys at 500° C.

| Alloy Analysis, w/o | Tensile Properties at 500° C.                        |                                         |                                        |                                            |                               |
|---------------------|------------------------------------------------------|-----------------------------------------|----------------------------------------|--------------------------------------------|-------------------------------|
|                     | Yield<br>Strength<br>(0.2% Offset)<br>1,000 p. s. i. | Ultimate<br>Strength,<br>1,000 p. s. i. | Elongation to<br>Max. Load,<br>Percent | Total Elonga-<br>tion in 1 in.,<br>Percent | Reduction of<br>Area, Percent |
| 1.0 Nb+0.5 Al       | 26.5                                                 | 39.3                                    | 10                                     | 30                                         | 31                            |
| 1.5 Nb+1.0 Al       | 34.3                                                 | 44.7                                    | 6                                      | 27                                         | 31                            |
| 1.8 Nb+0.6 Mo       | 17.8                                                 | 28.8                                    | 8                                      | 39                                         | 30                            |
| 1.4 Nb+1.1 Mo       | 20.9                                                 | 32.5                                    | 4                                      | 40                                         | 43                            |
| 2.0 Nb+1.6 Mo       | 29.3                                                 | 38.4                                    | 2                                      | 42                                         | 48                            |
| 1.0 Nb+0.3 V        | 16.5                                                 | 28.6                                    | 6                                      | 30                                         | 39                            |
| 1.3 Nb+1.1 V        | 20.5                                                 | 32.7                                    | 7                                      | 21                                         | 26                            |
| 2.2 Nb              | 35                                                   | 43                                      |                                        | 9                                          | 15                            |
| 6.0 Nb              | 36.3                                                 | 52.4                                    | 3                                      | 8                                          | 5                             |

The data of the above table graphically illustrate the great increase in ductility which is obtained in the ternary alloys of the present invention over the binary zirconium-niobium alloys without any sacrifice in yield strength.

The improved characteristics of the alloys of this invention for high-temperature reactor structural materials may best be illustrated by comparing the yield strength

60 1.5 weight percent niobium, 1.0 weight percent aluminum, and zirconium and characterized by having a thermal neutron capture cross section of 0.19 barn per atom and a 0.2% offset yield strength at 500° C. of 34,300 p. s. i.

## References Cited in the file of this patent

Schwope et al.: Journal of Metals, November 1952, pages 1138-1140.